

## UNITED STATES PATENT OFFICE

WILLIAM THEODORE ANDERSON, JR., AND LESTER FLETCHER BIRD, OF NEWARK, NEW JERSEY, ASSIGNEES TO HANOVIA CHEMICAL AND MANUFACTURING COMPANY, OF NEWARK, NEW JERSEY, A CORPORATION OF NEW JERSEY

## PROCESS FOR CUPRIC-OXIDE REMOVAL

No Drawing.

Application filed October 28, 1927. Serial No. 229,524.

This invention relates to a process for the removal of cupric oxide (black) from the surfaces of crystalline cuprous oxide or from the surfaces of metallic copper.

5 The removal of the black oxide can be accomplished by mechanical means for example by planing or cutting with abrasives such as emery cloth or cutting wheels but very often such methods are not desirable. In 10 those cases where it is necessary to remove black oxide from the surface of red oxide it is very important that the red oxide should not be damaged or broken in any way. Since the black oxide is harder than the red oxide 15 any device that will remove the black oxide will readily remove the red oxide as well. Our invention as herein described and defined in the appended claim sets forth a process which we have found to be very de- 20 sirable and effective in removing black cupric oxide from copper or cuprous oxide surfaces. This process will not produce mechanical damage, such as cracks or abrasions, to the under surfaces and will remove any thick- 25 ness of black oxide ordinarily produced in the treatment of copper.

The cupric (black) oxide as formed on copper surfaces or on top of red oxide surfaces is of fine crystalline structure and is 30 quite porous to liquids or gases. The red cuprous crystalline oxide on the other hand is attacked comparatively slowly by either liquids or gases. These characteristics are favorable to electrolytic methods of separa- 35

The electrolyte required by our process may be dilute sulphuric acid or other strong acid which readily attacks copper oxides. Any variety or concentration of copper salts 40 may be included in the electrolyte. The copper plate covered with oxide is used for an electrode in this electrolyte and a piece of pure copper or chemically inert conducting substance for the other electrode. If direct 45 current is passed through the solution in either direction reduction of the surface oxide occurs. If the oxide coated copper is made the cathode a deposit of metallic spongy copper is formed replacing the reduced oxide on the surface. Copper so

formed can be removed by reversing the direction of current flow. Alternating current is the more desirable electrical supply since by its use the oxide is loosened without any deposition of metallic copper. After several 4 seconds of treatment the loosened oxide can be washed off leaving the under surface clean. Further action by the acid, after the cleaned surface is removed from the solution, is prevented by immediate neutralization with an alkaline substance, for example, dipping the cleaned surface in a dilute solution of ammonium hydroxide. 60

The advantages of this process are many. First, a satisfactory simple cleaning method 65 removes the need for special precautions to prevent the formation of the black oxide on the surfaces. Second, all parts of the process are simple requiring no special or elaborate equipment. Third, only the black oxide is 70 attacked readily by this procedure, since the red crystalline oxide is only acted upon at a greatly reduced rate. Fourth, the black oxide is completely loosened from the surface so that it can be washed off entirely with a 75 minimum of labor. Fifth, the concentration of electric current is not important and may vary widely. Sixth, the kind or type of electrolyte is not critical and many kinds and concentrations are suitable. 80

Having described our invention, what we claim as new and desire to secure by Letters Patent, is:—

The herein described process of removing cupric oxide from a metallic copper and crystalline cuprous oxide surface, which consists in placing the object carrying the cupric oxide into an electrolyte, said electrolyte being a strong acid which readily attacks copper oxide, passing an alternating electric current through the electrolyte to the cupric oxide as an electrode to thereby loosen the cupric oxide, washing off the loosened cupric oxide from the object, and then immersing the object in an alkaline substance to prevent 95 further action of the acid. 85

This specification signed and witnessed this twenty-fifth day of October, 1927.

WILLIAM THEODORE ANDERSON, Jr.  
LESTER FLETCHER BIRD.